

## UNITED STATES PATENT OFFICE

2,388,368

## IGNITION COMPOSITION

Guy F. Rolland, McKeansburg, Pa., assignor to  
 Atlas Powder Company, Wilmington, Del., a  
 corporation of Delaware

No Drawing. Application May 6, 1941,  
 Serial No. 392,183

9 Claims. (Cl. 52—2)

This invention relates to improved ignition compositions, and more particularly to the improvement of ignition compositions which comprise a metallic acetylide and to a method of improving the stability and reliability of metallic acetylide ignition compositions. It has for its main object the improvement of the inflammability, stability and reliability of such ignition compositions after prolonged storage periods. Other objects will also be evident from the following description of my invention.

Ignition compositions comprising an inflammable metallic acetylide such as, for example, cuprous acetylide, mercury acetylide and silver acetylide are useful for many purposes and particularly where the ignition composition is to be ignited by electrical means, such as, for example, electrically heated bridge wires, spark gaps, etc. They are adaptable and greatly valued for use, for example, in electric detonators, electric squibs, electric starter cartridges, electrically fired coal blasting devices, oil-well casing perforators, etc., as is well known. For such purposes, cuprous acetylide in particular is highly desirable because it is readily ignited by means of a relatively small amount of heat and burns with a quick but relatively non-violent flash. One objection to cuprous acetylide has always existed, however, in that it has had a tendency to lose its sensitivity to low temperature ignition as well as its desirable flash characteristics, after prolonged storage periods and particularly when stored under conditions involving elevated temperatures. The rate of deterioration of cuprous acetylide, under fixed storage conditions, has varied widely among different manufactured lots of the materials, some lots even showing a marked decrease in sensitivity with as little as three months storage at a temperature of 50° C. while other lots show little or no deterioration over much longer periods under the same storage conditions.

The lots which exhibit marked decrease in sensitivity, as evidenced, for example, by their decreased sensitivity to ignition by the heated bridge wire of an electric match, are unsuitable for use as ignition compositions. Consequently, it is necessary, before a lot of cuprous acetylide is made into matches or the like, to store it for extensive periods, as, for example, from two to three months, in order to determine whether or not it has the undesirable characteristic of reduction in sensitivity with aging.

Now, in accordance with the present invention, I overcome this objection by greatly prolonging

the inflammation-sensitivity life of the metallic acetylide by associating with it a stabilizer comprising abietic acid. A typical example of such a stabilizer is rosin, as obtained, for example, from the distillation of turpentine oil from crude turpentine, which product I have found to be very effective in improving the storage life of metallic acetylide types of ignition compositions, when intimately associated therewith, even in very small proportions.

It is customary to apply the acetylide, such as, for example, cuprous acetylide, to the bridge wire or other heat-producing means in the form of a suspension in nitrocellulose lacquer. A commonly used solvent for such lacquer is amyl acetate, although other suitable solvents may be employed. Also, the lacquer may comprise binders other than nitrocellulose. The stabilizer (abietic acid or composition comprising this material) may be conveniently dissolved in the lacquer, in which the acetylide is to be suspended. The stabilizer may also be added to the acetylide-lacquer mixture in the form of an amyl acetate solution. Either method of application insures an intimate mixture of the acetylide and abietic acid stabilizer when the solvent has evaporated from the mixture. After the lacquer mixture has been applied to a bridge wire, for example, (usually by dipping the device into the mixture), the lacquer solvent is allowed to evaporate, resulting in the formation of a coherent bead of heat sensitive composition about the bridge wire or other heat producing device. The electric ignition device may then be completed in any manner desired, as by successive applications of protecting lacquer, by applying an auxiliary flame-producing mixture which may consist, for example, of a mixture of charcoal and potassium chlorate suspended in lacquer, etc., the solvent being allowed to evaporate between each application of material to the assembly. Well-known devices of this type are known as fuse-heads or match-heads.

A non-limiting example of an ignition composition of the present invention is as follows:

45 Cuprous acetylide..... 75 grams  
 Rosin, grade N..... 1.92 grams—dissolved in  
 Nitrocellulose lacquer  
 (1½ oz. per gallon)..... 63.5 ml.

10 The amount of stabilizer in the above example corresponds to 2.5% of the dry material, exclusive of the nitrocellulose in the lacquer. However, this proportion of stabilizer is not critical and it is to be understood that even smaller amounts

may be employed with good effect. Also, larger amounts may be employed, although it is desirable not to replace too much of the cuprous acetylid with rosin, since the cuprous acetylid is the active inflammable ingredient of the ignition composition. Generally, I have found that amounts of rosin up to 5% will have no materially adverse effect on the firing characteristics of the acetylid composition. In general, therefore, the stabilizer of the composition of the present invention is present in amounts small enough to be effective in increasing the stability of the inflammable metallic acetylid without adversely affecting the firing characteristics of the acetylid. The amount of lacquer used may vary considerably depending on the character of the particular cuprous acetylid used. The actual amount used is such as to obtain proper consistency for application to the bridge wire. The grade of rosin used need not be that indicated above but may be any of the other grades of rosin, as well as pure abietic acid.

The effectiveness of the stabilizer is shown by the following sensitivity tests on match heads made with the composition of the above example, as compared with sensitivity tests on match heads made from the same lot of cuprous acetylid but with no stabilizer present, the assembly of the matches being otherwise identical.

|                                                | Sensitivity of ignition compositions on matched heads |                        |
|------------------------------------------------|-------------------------------------------------------|------------------------|
|                                                | As manufactured                                       | After 3 mos. at 50° C. |
| Cuprous acetylid stabilized with grade N rosin | Ma. 270                                               | Ma. 275                |
| Cuprous acetylid with no stabilizer            | 260                                                   | 305                    |

The sensitivity of the ignition composition on the match heads was determined by measuring the minimum amount of current through the bridge wire required to cause consistent ignition of the composition. The higher minimum current requirement in the above tabulation indicates a lower sensitivity. The increase in current requirement of the unstabilized cuprous acetylid indicates that deterioration had already begun, whereas the current requirements for the stabilized material was identical, within experimental limits of error, after the storage period, indicating continued good sensitivity.

It will therefore be evident, that by means of the present invention, I provide not only greater storage life to ignition compositions comprising inflammable metallic acetylid, resulting in a

more uniformly low minimum firing current therein, and thereby greatly increasing the functioning reliability after storage, but I also provide a means of maintaining a more uniform minimum firing current from batch to batch of inflammable metallic acetylid, irrespective of its age. This latter feature serves to insure better series firing characteristics and particularly where ignition devices of various ages are connected in the same series circuit.

It is to be understood that the ignition compositions of the present invention may comprise ingredients other than those mentioned above, as, for example, fuels, oxidizers, etc., without departing from the present invention.

The above example and test results are cited merely for purposes of fully illustrating the invention and are not to be considered as limiting.

Having described my invention, what I claim is:

1. An ignition composition comprising a mixture of a metallic acetylid and a stabilizer comprising abietic acid.
2. An ignition composition comprising a mixture of cuprous acetylid and a stabilizer comprising abietic acid.
3. An ignition composition comprising a mixture of a metallic acetylid and a stabilizer consisting essentially of rosin.
4. An ignition composition comprising a mixture of cuprous acetylid and a stabilizer consisting essentially of rosin.
5. In an electric ignition device, an electrically heated bridge wire in direct contact with an inflammable ignition composition comprising a mixture of cuprous acetylid and a stabilizer comprising abietic acid.
6. In an electric ignition device, an electric spark gap having within the gap and adapted to become ignited by a spark passing through the gap, an inflammable ignition composition comprising a mixture of cuprous acetylid and a stabilizer comprising abietic acid.
7. In combination in an ignition device an inflammable ignition composition comprising a mixture of a metallic acetylid and a stabilizer comprising abietic acid, and a heat-producing means positioned to ignite said composition.
8. In combination in an ignition device an inflammable ignition composition comprising a mixture of cuprous acetylid and a stabilizer comprising abietic acid, and a heat-producing means positioned to ignite said composition.
9. An ignition composition comprising a mixture of a metallic acetylid, a stabilizer comprising abietic acid, and a binder.

GUY F. ROLLAND.